

# United States Patent Office

2,835,581

Patented May 20, 1958

1

2,835,581

## TETRAZAINDENES AND PHOTOGRAPHIC EMULSIONS CONTAINING THEM

John F. Tinker and John Sagal, Jr., Rochester, N. Y., assignors to Eastman Kodak Company, Rochester, N. Y., a corporation of New Jersey

No Drawing. Application June 15, 1955

Serial No. 515,785

9 Claims. (Cl. 96—109)

This invention relates to fog inhibiting agents and stabilizers for photographic emulsions and to photographic emulsions containing them.

It is well known that photographic emulsions on storage tend to lose sensitivity and to become spontaneously developable without exposure to light. There is normally a detectable amount of the silver salt reduced during development in the areas where no exposure was given; this is commonly called "fog," and sometimes called "chemical fog" where it is necessary to distinguish between it and the effects of accidental exposure to radiation; in this invention, we are not concerned with the latter.

Fog depends both on the emulsion and the conditions of development; for a given emulsion it increases with the degree of development. With constant development conditions, it tends to increase with time, temperature and relative humidity of storage conditions; it is common practice to make accelerated tests of the stability of photographic emulsions by storage at increased temperature or humidity, or both. It is, of course, desirable to have emulsions as stable as possible under the conditions of high temperature and humidity which may occur in tropical climates, for example. Fog usually appears over the whole area of the sensitive coating, but when severe, it frequently is non-uniform. Fog may also be caused by exposure to chemicals, for example, hydrogen sulfide and other reactive sulfur compounds, hydrogen peroxide vapor, and strongly reducing materials. While anti-foggants and stabilizers may protect, to some extent, against such effects, it is normally understood that an antifogulant protects against spontaneous growth of fog during prolonged storage or storage at high temperatures and humidities, or during development to maximum contrast and speed, or both.

It is, therefore, an object of the present invention to provide a method for stabilizing photographic emulsions. A further object is to provide a means for reducing the fog produced upon keeping of such emulsions which have been sensitized, especially emulsions stored under tropical or other adverse conditions. A still further object is to provide a means for stabilizing the speed and contrast of sensitized photographic emulsions. Other objects will become apparent from a consideration of the following description and examples.

According to our invention, we provide a method for stabilizing photographic silver halide emulsions by incorporating therein a compound selected from those represented by the following general formula:



wherein R represents a hydroxyl group or a halogen atom, such as chlorine, bromine, etc., R<sub>1</sub> represents an alkyl group (such as a methyl group, etc.), an aryl group (such as phenyl, p-methoxyphenyl, etc., especially a mononuclear aromatic group of the benzene series), or a heterocyclic group (such as 2-pyridyl, 2-furyl, etc.),

2

and R<sub>2</sub> represents a hydrogen atom, an alkyl group (such as methyl, ethyl, etc.), or an aryl group (such as phenyl, tolyl, etc., especially a mononuclear aromatic group of the benzene series). The compounds

represented by Formula I above wherein R<sub>1</sub> represents a methyl group and R<sub>2</sub> represents a hydrogen atom have been found to be especially useful in practicing our invention. The compounds selected from those represented by Formula I above (R is hydroxyl) can advantageously be prepared by condensing 3-amino-5-hydroxy-methyl-1,2,4-triazole together with an ester selected from those represented by the following general formula:

(II)



wherein R<sub>1</sub> and R<sub>2</sub> each has the values given above and R<sub>3</sub> represents a lower alkyl group (such as methyl, ethyl, etc.). Such a method has been previously described in Heimbach and Kelly U. S. Patent 2,444,604, issued July 6, 1948, and "Berichte," vol. 42, page 4643, and vol. 43, pages 378-380. The compounds selected from those represented by Formula I above wherein R is a halogen atom can advantageously be prepared by heating together a compound selected from those represented by

Formula I above wherein R is a hydroxyl group and a phosphoryl halide, such as phosphoryl chloride. Illustrative examples of these methods are given below.

Compounds selected from those represented by Formula I above which can be used in our invention include those represented by the following formulas:

(1)



35

4-hydroxy-2-hydroxymethyl-6-methyl-1,3,3a,7-tetraazaindene

(2)



40

2-chloromethyl-4-hydroxy-6-methyl-1,3,3a,7-tetraazaindene

(3)



45

4-hydroxy-2-hydroxymethyl-6-phenyl-1,3,3a,7-tetraazaindene

(4)



50

5-ethyl-4-hydroxy-2-hydroxymethyl-6-methyl-1,3,3a,7-tetraazaindene

(5)



55

2-chloromethyl-4-hydroxy-6-phenyl-1,3,3a,7-tetraazaindene

(6)



60

4-hydroxy-2-hydroxymethyl-6-methyl-5-phenyl-1,3,3a,7-tetraazaindene

The antifoggant compounds represented by Formula I can be employed in emulsions which have been sensitized optically or chemically, or emulsions which have not been so sensitized. It is known that the effective sensitivity of photographic silver halide emulsions can be increased by adding to them derivatives of alkylene oxides, such as ethylene oxide polymers having molecular weights of 300 or more. The practical value of these compounds is severely limited by their tendency to increase fog on storage of the photographic film, especially storage at elevated temperatures and humidity. It has been found difficult to control this by the antifoggants commonly available without using quantities of antifoggants which partly neutralize the speed increase obtained from the alkylene oxide derivatives.

The alkylene oxide polymers used to sensitize the emulsions can be of various types. The alkylene oxides from which the polymers are derived contain from 2 to 4 carbon atoms, e. g., ethylene oxide, propylene oxide and butylene oxide. The preparation of polymers from these compounds is described in Ellis, *The Chemistry of Synthetic Resins* (1935), pages 990 to 994. These compounds are also referred to as polyalkylene glycols and their use as sensitizers for silver halide emulsions is described in U. S. Patents 2,423,549 and 2,441,389. Ethylene oxide polymers have been found to be especially advantageous in practicing our invention.

Various derivatives of alkylene oxides may also be used to sensitize the silver halide emulsions, e. g., condensation products of alkylene oxide with glycols, such as those having from 8 to 18 carbon atoms, as described in U. S. Patent 2,240,472 and British Patent 443,559, as well as condensation products of alkylene oxides with aliphatic alcohols, aliphatic acids and aliphatic amines, that is, polyalkylene ethers, esters and amides, the preparation of which is described in U. S. Patent 1,970,578, condensation products of alkylene oxides with phenols, also described in U. S. Patent 1,970,578, and condensation products of alkylene oxides with hexitol ring dehydration products, as described in U. S. Patent 2,400,532.

In each case the polyalkylene oxide or derivative of alkylene oxide should have a molecular weight of at least 300. Condensation products of ethylene oxide with long chain alcohols should have a molecular weight of about 700; other derivatives may have a molecular weight of 1500 to 4000 or more.

The principal purpose of our invention is to provide a means for maintaining the sensitivity and fog of silver halide emulsions at or close to initial optimum values under conditions of high temperature or high humidity, or both. Preferably, the antifoggants of our invention are added to the emulsion at any stage during the process of manufacture prior to coating the emulsion. The antifoggants can be added to the emulsion in solution in water or any convenient solvent not injurious to the emulsion, such as lower aliphatic alcohols.

The solutions of antifoggants which we employ when added in suitable concentration before coating to unsensitized or optically sensitized silver halide emulsions usually do not appreciably affect the sensitivity and fog when measurements are made soon after coating. However, when sensitometric measurements are made after appreciable intervals of time under tropical or dry conditions of storage at elevated temperatures, the antifoggants do stabilize speed and maintain fog at a low level.

The alkylene oxide derivatives which can be used to sensitize the emulsions can be illustrated by the following specific examples, although our invention is in no way limited to the use of these specific compounds.



Polyethylene oxide



Di-(polyethylene-glycoxy)-decane



Polyethylene oxide oleyl ether

where  $n$  = an integer greater than about 10.

The preparation of silver halide emulsions involves three separate operations: (1) the emulsification and digestion or ripening of the silver halide, (2) the freeing of the emulsion from aqueous soluble salts usually by washing, (3) the second digestion or after-ripening to obtain increased sensitivity (Mees, *The Theory of the Photographic Process*, 1942, page 3). The fog inhibiting agents can be added at any stage, preferably after the final digestion.

The photographic emulsions which we use are of the developing-out type and best results have been obtained with gelatino-silver bromoiodide emulsions. However, emulsions of varying halide content can be used.

The emulsions can be chemically sensitized by any of the accepted procedures. The emulsions can be digested with naturally active gelatin, or sulfur compounds may be added such as those described in Sheppard U. S. Patent 1,574,944 and U. S. 1,623,499, and Sheppard and Brigham U. S. Patent 2,410,689.

The emulsions can also be treated with salts of the noble metals such as ruthenium, rhodium, palladium, iridium and platinum, all of which belong to group VIII of the periodic table of elements and have an atomic weight greater than 100. Representative compounds are ammonium chloropalladate, potassium chloroplatinate and sodium chloropalladite, which are used for sensitizing in amounts below that which produces any substantial fog inhibition, as described in Smith and Trivelli U. S. Patent 2,448,060, and as antifoggants in higher amounts, as described in Trivelli and Smith U. S. Patents 2,566,245 and 2,566,263.

The emulsions can also be chemically sensitized with gold salts as described in Waller and Dodd U. S. Patent 2,399,083, or stabilized with gold salts as described in Damschroder U. S. Patent 2,597,856 and Yutzy and Leermakers U. S. Patent 2,597,915. Suitable compounds are potassium chloroaurite, potassium aurithiocyanate, potassium chloroaurate, auric trichloride and 2-aurosulfobenzothiazole methochloride.

The emulsions can also be chemically sensitized with reducing agents, such as stannous salts (Carroll U. S. Patent 2,487,850), polyamines such as diethylene triamine (Lowe and Jones U. S. Patent 2,518,698), polyamines such as spermine (Lowe and Allan U. S. Patent 2,521,925), or bis-( $\beta$ -aminoethyl) sulfide and its water-soluble salts (Lowe and Jones U. S. Patent 2,521,926).

The emulsions can also be stabilized with the mercury compounds of Allen, Byers and Murray U. S. application Serial No. 319,611 (now U. S. Patent 2,728,663, issued December 27, 1955); Carroll and Murray U. S. application Serial No. 319,612 (now U. S. Patent 2,728,664, issued December 27, 1955); and Leubner and Murray U. S. application Serial No. 319,613 (now U. S. Patent 2,728,665, issued December 27, 1955), all filed November 8, 1952.

The antifoggants of our invention alone, or in combination with polyalkylene oxides or their derivatives, are effective in the presence or absence of optical sensitizing dyes. Since optical sensitizing can affect stability of emulsions with respect to sensitivity, fog and latent image changes, the action of the antifoggants is not completely independent of optical sensitizing or other emulsion variables. We have found, however, that both un-

sensitized emulsions and emulsions sensitized with cyanine or merocyanine dyes, or both, can be treated with the antifogging compounds represented by Formula I above.

The quantity of antifoggant compound employed can be varied, depending upon the particular silver halide employed, degree of ripening, presence or absence of other emulsion addenda, etc. In general, the quantity of antifoggant can vary from about 0.1 to 10 grams per gram mole of silver halide in the emulsion. These amounts can be used in combination with one or more of the chemical sensitizing and stabilizing agents listed above.

The stabilizing action afforded by the antifoggants of our invention was determined by incubation of the emulsions for a period of two weeks at 120° F. and at constant humidity. The speeds were measured in terms of 30/E where E is the exposure required to produce a density of 0.2 above fog. The antifoggants were added to a panchromatically sensitized, high speed silver bromoiodide emulsion which had been chemically sensitized with a sulfur compound, such as described in Sheppard U. S. Patent 1,574,944 and potassium chloroaurate. The emulsions were coated on a cellulose acetate support and the coatings exposed ( $\frac{1}{25}$ ") on an Eastman I(b) Sensitometer and processed for four minutes in a developer (Kodak D-19) having the following composition:

|                                |    |      |
|--------------------------------|----|------|
| Water, about 125° F            | cc | 500  |
| N-methyl-p-aminophenol sulfate | g  | 2.0  |
| Sodium sulfite, desiccated     | g  | 90.0 |
| Hydroquinone                   | g  | 8.0  |
| Sodium carbonate, monohydrate  | g  | 52.5 |
| Potassium bromide              | g  | 5.0  |
| Cold water to make one liter.  |    |      |

Alternatively, the exposed coatings were processed for five minutes in Kodak DK-50 developer, having the following composition:

|                                |      |
|--------------------------------|------|
| N-methyl-p-aminophenol sulfate | 2.5  |
| Hydroquinone                   | 2.5  |
| Sodium sulfite, desiccated     | 30.0 |
| Sodium metaborate              | 10.0 |
| Potassium bromide              | 0.5  |
| Water to make one liter.       |      |

The results of these tests for speed, gamma and fog, before and after incubation of each of the samples, are given in the following table. In the table, the same batch of emulsion was employed in Examples 1 and 2, the same batch of emulsion was employed in Examples 3 and 4 and the same batch of emulsion was employed in Examples 5 and 6.

In a manner similar to that illustrated in the above examples, other compounds selected from those represented by Formula I can be used to stabilize photographic silver halide emulsions, either in the presence or absence of chemical sensitizers.

We have also found that compounds corresponding to those of Formula I wherein R represents a formamidinothio (hydrochloride) group can be employed in photographic silver halide emulsions, though less advantageous than the compounds represented by Formula I.

Instead of incorporating the antifoggants in the photographic silver halide emulsion, these antifoggants can be incorporated in a colloid layer, such as a gelatin overcoating layer or interlayer, in contact with the emulsion.

The fog-inhibiting agents which we have described can be used in various kinds of photographic emulsions. In addition to being useful in non-sensitized emulsions, they can also be used in orthochromatic, panchromatic, and

X-ray emulsions. If used with sensitizing dyes they can be added to the emulsion before or after the dyes are added. Various silver halides can be used as the light-sensitive material, including silver bromide, silver iodide, silver chloride, silver bromoiodide, silver chlorobromide, silver chlorobromiodide, etc. The antifogants of our invention can be used in emulsions intended for color photography, for example, emulsions containing color-forming couplers, or emulsions to be developed by solutions containing couplers.

The polyethylene oxide polymers used in the emulsions according to our invention can be prepared either by polymerizing ethylene oxide in the presence of aliphatic acids, aliphatic amines, or phenols, or by reacting the polymerized polyethylene oxide with aliphatic acids, acid chlorides, or esters, which produces similar products.

The dispersing agents can be gelatin, or other colloids, such as collodion, albumen, cellulose derivatives, synthetic resins, etc.

The following examples will illustrate the method referred to above of preparing the compounds of Formula I, or the corresponding compounds wherein R is a formamidinothio group. Other somewhat similar compounds are shown in Examples 12 and 13 below.

**Example 7.—3-amino-5-hydroxymethyl-1,2,4-triazole**



50 A mixture of 272 g. (two moles) of aminoguanidine bicarbonate, 440 ml. of 70 percent aqueous glycolic acid (four moles), and two ml. of concentrated nitric acid was refluxed for 24 hours, then cooled well and filtered.

TABLE I

| Example | Compound | Concen-<br>tration<br>per Mole<br>AgX, g. | Devel-<br>oper Em-<br>ployed | Fresh Tests   |       |      | 2 Wks., 120° F. |       |      |     |
|---------|----------|-------------------------------------------|------------------------------|---------------|-------|------|-----------------|-------|------|-----|
|         |          |                                           |                              | Rel.<br>Speed | Gamma | Fog  | Rel.<br>Speed   | Gamma | Fog  |     |
|         |          |                                           |                              |               |       |      |                 |       |      |     |
| 1       | (a)      | Control                                   | D-19                         | 3,150         | 1.49  | .14  | 2,850           | 1.16  | .23  |     |
|         |          | (A)                                       | do                           | 3,600         | 1.47  | .12  | 3,350           | 1.31  | .18  |     |
|         |          | (A)                                       | do                           | 3,850         | 1.44  | .11  | 3,600           | 1.32  | .14  |     |
| 2       | (d)      | (B)                                       | 0.75                         | do            | 4,750 | 1.10 | .14             | 5,450 | 0.94 | .24 |
|         |          | (B) plus                                  | 0.75                         | do            | 4,750 | 1.04 | .14             | 5,700 | 0.91 | .10 |
|         |          | (A)                                       | 0.9                          | do            | 8,650 | 0.82 | .14             | 8,450 | 0.66 | .11 |
| 3       | (f)      | Control                                   | DK-50                        | 5,850         | 0.94  | .20  | 5,200           | 0.80  | .20  |     |
|         |          | (A)                                       | do                           | 6,150         | 0.92  | .11  | 5,600           | 0.81  | .17  |     |
|         |          | (B)                                       | 0.75                         | do            | 8,250 | 0.86 | .15             | 6,250 | 0.63 | .24 |
| 4       | (i)      | (B) plus                                  | 0.75                         | do            | 8,650 | 0.79 | .14             | 7,700 | 0.61 | .14 |
|         |          | (A)                                       | 0.9                          | do            | 8,650 | 0.79 | .14             | 7,700 | 0.61 | .14 |
|         |          | (B) plus                                  | 0.75                         | do            | 8,650 | 0.79 | .14             | 7,700 | 0.61 | .14 |
| 5       | (k)      | Control                                   | D-19                         | 3,600         | 1.30  | .16  | 3,600           | 1.12  | .20  |     |
|         |          | (C)                                       | 0.9                          | do            | 3,850 | 1.43 | .14             | 3,700 | 1.12 | .17 |
|         |          | (B)                                       | 0.75                         | do            | 5,200 | 1.21 | .21             | 6,250 | 0.88 | .27 |
| 6       | (m)      | (B) plus                                  | 0.75                         | do            | 5,450 | 1.25 | .16             | 5,850 | 1.03 | .21 |
|         |          | (C)                                       | 0.9                          | do            | 5,450 | 1.25 | .16             | 5,850 | 1.03 | .21 |

In the above table: A = 4-hydroxy-2-hydroxymethyl-6-methyl-1,3,3a,7-tetraazaindene; B = polyethylene glycoether of oleyl alcohol; C = 2-chloromethyl-4-hydroxy-6-methyl-1,3,3a,7-tetraazaindene.

The solid was boiled with 500 ml. of 95 percent ethanol, filtered (the insoluble material discarded) and cooled. The precipitated solid, 114 g. or 50 percent, melted at 94–102° C., but was pure enough for use in the next step. This compound crystallized as a salt of glycolic acid; one sample, crystallized several times from ethanol, M. P. 114–115° C., corresponds nearly to the 1:1 compound. Evidently, the glycolic acid was gradually removed by crystallization from ethanol.

*Analysis.*—Calc'd for  $C_3H_6N_4O.C_2H_4O_3$ : C, 31.5; H, 5.3; N, 29.5. Found: C, 32.0; H, 5.3; N, 31.4.

*Example 8.—4-hydroxy-2-hydroxymethyl-6-methyl-1,3,3a,7-tetrazaindene*



A mixture of 50 g. of the compound described above (Example 7), 5 ml. of glacial acetic acid, and 250 ml. of ethyl acetoacetate was heated on the steam cone overnight. Cooled, filtered, and the solid recrystallized from 400 ml. of 6 N hydrochloric acid; 50 g., 63 percent, of solid, M. P. 268–270° C. were obtained.

*Analysis.*—Calc'd: C, 46.6; H, 4.5; N, 31.1. Found: C, 45.8; H, 4.8; N, 31.1.

Crystallization from water yielded the hemihydrate, M. P. 227–229° C.

*Analysis.*—Calc'd: C, 44.5; H, 4.8; N, 29.7. Found: C, 44.5; H, 4.7; N, 29.8.

*Example 9.—2-chloromethyl-4-hydroxy-6-methyl-1,3,3a,7-tetrazaindene*



Twenty-five g. of the substance described above (Example 8) was refluxed with phosphoryl chloride for one hour, evaporated to dryness at 90° C. and 20 mm., and treated with ice water. The mixture was treated with a little cyclohexanone and some chloroform, and allowed to warm up to room temperature during several hours, after which the product, at first gluey, had become a white powder. It was filtered and dried; 13.8 g., 48 percent, of the hemihydrate, M. P. 260–263° C., was obtained.

*Analysis.*—Calc'd for  $C_3H_6ClN_4O.1/2H_2O$ : C, 40.6; H, 3.9; Cl, 17.2; N, 27.1. Found: C, 39.5; H, 3.9; Cl, 17.4; N, 27.9.

Crystallization from 6 N hydrochloric acid yielded the anhydrous compound, M. P. 265–266° C.

*Analysis.*—Calc'd: C, 42.4; H, 3.5; Cl, 17.9; N, 28.2. Found: C, 42.4; H, 3.7.

*Example 10.—2-formamidinothiomethyl-4-hydroxy-6-methyl-1,3,3a,7-tetrazaindene*



Two grams of 2-chloromethyl-4-hydroxy-6-methyltetrazaindene and one gram of thiourea in 100 cc. of ethanol were refluxed 8 hours. Three hundred cc. more alcohol were added, heated to boiling, and filtered. The residue recrystallized from 70 cc. of aqueous ethanol, yielding 0.6 gram, M. P. 262–264° C. dec.

*Analysis.*—Calc'd:  $C_8H_{13}ClN_6O_2S$  (m. wt. 293): C, 32.8; H, 4.4; N, 29.4; S, 11.0. Found: C, 33.3; H, 4.6; N, 29.4; S, 11.3.

8  
*Example 11*

4-chloro-2-chloromethyl-6-methyl-1,3,3a,7-tetrazaindene was produced by reacting 4-hydroxy-2-hydroxymethyl-6-methyltetrazaindene with phosphorous oxychloride as described above, and carefully decomposing the residue (from removal of excess phosphorus oxychloride) with ice. The material was a yellow solid, M. P., about 181° C.; it was not obtained pure. Recrystallization from water converted it to 2-chloromethyl-4-hydroxymethyl-6-methyltetrazaindene, M. P., 266–269° C.

*Example 12.—2-chloromethyl-6-methyl-4-morpholino-1,3,3a,7-tetrazaindene*



A mixture of 20 grams of the crude dichloro derivative, (Example 11), 350 cc. of ethanol, and 18 cc. of morpholine was refluxed 2 hours; enough water was added to give complete solution, then filtered and cooled. A white solid separated, 11 grams, 47 percent, M. P., 204–205° C.

*Analysis.*—Calc'd:  $(C_{11}H_{14}ClN_5O$ , m. wt. 268): C, 49.4; H, 5.2. Found: C, 49.5, 49.1; H, 5.3, 5.7.

*Example 13.—Bis(2-formamidinothiomethyl-6-methyl-1,3,3a,7-tetrazainden-4-yl)-sulfide dihydrochloride dihydrate*



A mixture of 20 grams of the dichloro derivative (Example 11), 7.7 grams of thiourea, and 350 cc. of ethanol was refluxed 2 hours; evaporated to dryness, crystallized from ethanol-ethyl acetate, then several times from ethanol, finally yielding 2.2 grams of pale yellow solid, M. P., 144–145° C. (9 percent yield).

*Analysis.*—Calc'd:  $(C_{18}H_{24}Cl_2N_2S_3O_2$ , m. wt. 582): C, 33.0; H, 4.1; N, 28.9; S, 16.5. Found: C, 34.0; H, 3.8; N, 28.9; S, 16.7.

What we claim as our invention and desire secured by Letters Patent of the United States is:

1. A photographic silver halide emulsion containing a compound selected from those represented by the following general formula:



65 wherein R represents a member selected from the group consisting of a hydroxyl group and a chlorine atom,  $R_1$  represents a member selected from the group consisting of a methyl group and a mononuclear aromatic group of the benzene series, and  $R_2$  represents a member selected from the group consisting of a hydrogen atom, an alkyl group containing from 1 to 2 carbon atoms, and a mononuclear aromatic group of the benzene series.

70 2. A photographic silver halide emulsion as defined in claim 1 wherein the silver halide is silver bromide.

75 3. A photographic silver halide emulsion containing a

compound selected from those represented by the following general formula:



wherein R represents a member selected from the group consisting of a hydroxyl group and a chlorine atom and R<sub>2</sub> represents a member selected from the group consisting of a hydrogen atom, and alkyl group containing from 1 to 2 carbon atoms, and a mononuclear aromatic group of the benzene series.

4. A photographic silver halide emulsion as defined in claim 4 wherein the silver halide is silver bromiodide.

5. A photographic silver halide emulsion containing 4-hydroxy - 2 - hydroxymethyl - 6 - methyl - 1,3,3a,7-tetrazaindene.

6. A photographic silver bromiodide emulsion containing 4 - hydroxy - 2 - hydroxymethyl - 6 - methyl - 1,3,3a,7-tetrazaindene.

7. A photographic silver halide emulsion containing 2-chloromethyl - 4 - hydroxy - 6 - methyl - 1,3,3a,7-tetrazaindene.

8. A photographic silver bromiodide emulsion containing 2 - chloromethyl - 4 - hydroxy - 6 - methyl - 1,3,3a,7-tetrazaindene.

9. A photographic silver halide emulsion sensitized with an alkylene oxide polymer selected from the class consisting of condensation products of an alkylene oxide

10

with aliphatic acids, condensation products of an alkylene oxide with aliphatic amines, and condensation products of an alkylene oxide with phenols, said alkylene oxide containing from 2 to 4 carbon atoms and said alkylene oxide polymer having a molecular weight of at least 300, said photographic emulsion containing as a fog inhibiting agent an azaindene compound selected from those represented by the following general formula:



15. wherein R represents a member selected from the group consisting of a hydroxyl group and a chlorine atom, R<sub>1</sub> represents a member selected from the group consisting of a methyl group and a mononuclear aromatic group of the benzene series, and R<sub>2</sub> represents a member selected from the group consisting of a hydrogen atom, an alkyl group containing from 1 to 2 carbon atoms, and a mononuclear aromatic group of the benzene series.

#### References Cited in the file of this patent

#### UNITED STATES PATENTS

|           |                 |                |
|-----------|-----------------|----------------|
| 2,407,204 | English et al.  | Sept. 3, 1946  |
| 2,449,225 | Heimbach et al. | Sept. 14, 1948 |
| 2,519,715 | Stewart         | Aug. 22, 1950  |
| 2,657,136 | Knott et al.    | Oct. 27, 1953  |
| 2,673,152 | Allen et al.    | Mar. 23, 1954  |